

J. H. YOUNG,  
PROTECTED METAL ARTICLE,  
APPLICATION FILED MAR. 26, 1921.

1,418,348.

Patented June 6, 1922.

FIG. 1.



FIG. 2.



*Inventor:*  
James Howard Young  
*By:*  
Jas. H. Chisholm  
*atty.*

# UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## PROTECTED METAL ARTICLE.

1,418,348.

Specification of Letters Patent. Patented June 6, 1922.

Application filed March 26, 1921. Serial No. 455,969.

To all whom it may concern:

Be it known that I, JAMES HOWARD YOUNG, a citizen of the United States, residing in Pittsburgh, in the county of Allegheny and State of Pennsylvania, have invented an Improvement in Protected Metal Articles, of which the following description in connection with the accompanying drawings, is a specification, like characters on the drawings representing like parts.

This invention relates to a protected metal article of that character in which an article of corrodible metal, such as iron or steel, is protected against corrosion by a layer of asphalt or like bituminous material alone or in conjunction with layers of fibrous material, such as asbestos, wool or other fibrous felts.

Protective metal articles of this character described are efficient against corrosion as long as the bituminous layer remains intact, but where the bituminous layer is exposed, it is subject to the deleterious action of light, heat, and atmospheric conditions; also to abrasion and other mechanical actions in handling, crating and shipping, and in some cases to injury by adhesion of one protected article to another.

The present invention has for its object to provide a protected metal article of the character described, which is provided with a protective covering of a modified fibrous material, which is tough, durable, weather-resisting, nontacky at temperatures around 140° F., more or less light and heat reflecting and capable of being painted with ordinary paints.

A modified fibrous material suitable for the purpose, is a cellulose paper treated with solutions of relatively non-corrodible metals in such manner as to incorporate the metals in the fiber and provide the same with the desirable characteristics above-mentioned.

Such treated paper may be designated as a metallized fiber, which is applied in sheet form to the hydrocarbonaceous layer on the metal article, while said layer is in a tacky condition and is thereby adhesively secured to the metal article.

Fig. 1 is a plan of a protected metal article embodying this invention, and

Fig. 2, a section on an enlarged scale on the line 2—2, Fig. 1.

Referring to the drawing, *a* represents an article of corrodible metal, such as iron or steel, which may be rigid or flexible and of any form, and which is herein represented as a metal sheet.

The metal article *a* is provided with a protective layer *b* of asphalt or hydrocarbonaceous material of like character, which may be applied in any suitable manner as by passing the article *a* through a bath of melted asphalt.

The asphalt or like layer *b* has applied to it while in a tacky condition, a layer *c* of metallized fiber, which is adhesively affixed to the metal article *a* by the asphalt or like layer *b*. The metallized fiber is a cellulose paper having incorporated therein, relatively non-corrodible metals such as copper, zinc and the like, and may be made by passing the paper through a bath of cupro-ammonium hydroxide of such strength that it has the power of dissolving or gelatinizing cellulose. As the paper is drawn through the bath, the fibers of the paper are acted upon by the solution in such way as to gelatinize the outside of the fibers. The paper is then passed under pressure between rolls which serve the purpose of compressing the gelatinized fibers together, thereby forming a substantially impervious sheet.

The sheets are then dried at a low temperature, which results in loss of water and ammonia gas, leaving the copper combined with the cellulose as so-called cupro-cellulose. Paper treated as described has been known to the trade as Willesdon paper.

Other processes are known for making paper of this type, in which copper, zinc or the like relatively non-corrodible metals are embodied, and the metal in the metallized fiber layer *c* in the drawings is represented by the stipple.

The metallized fibrous layer *c* is tough, water-resisting, rot-proof, durable, weather-resisting and is capable of being painted with ordinary paints, consequently it affords a highly efficient and inexpensive fibrous protecting layer for the bituminous layer *b*, whereby an inexpensive, efficient

and durable protected metal article may be produced, which will not stick together and which can be used in warm and cold climates.

5 Claim:

As an improved article of manufacture, a protected metal article comprising an article of corrodible metal, a layer of bitumi-

nous or like hydrocarbonaceous material covering said corrodible metal, and a layer 10 of metallized paper adhesively affixed to said hydrocarbonaceous material.

In testimony whereof, I have signed my name to this specification.

JAMES HOWARD YOUNG.